

# United States Patent [19]

Shimizu

[11] 3,803,832

[45] Apr. 16, 1974

[54] DIAL FOR WRIST WATCH AND A METHOD OF MAKING THE SAME

[76] Inventor: Noriaki Shimizu, 521-5, Imafuku, Ohaza, Saitamaken, Kawagoe, Japan

[22] Filed: Jan. 23, 1973

[21] Appl. No.: 326,023

[30] Foreign Application Priority Data

Feb. 1, 1972 Japan..... 47-11541

[52] U.S. Cl..... 58/127 B, 58/127 R

[51] Int. Cl..... G04b 29/00

[58] Field of Search..... 58/127 R, 127 B, 126 R, 58/126 A; 29/177, 470.1

[56] References Cited

UNITED STATES PATENTS

1,708,293 4/1929 Fitch ..... 58/127 B  
3,523,845 4/1970 Robertson..... 29/470.1 X

FOREIGN PATENTS OR APPLICATIONS

348,363 8/1960 Switzerland..... 58/127 B

Primary Examiner—Stephen J. Tomsky

Assistant Examiner—U. Weldon

[57]

## ABSTRACT

A dial for a wrist watch comprises a dial body formed of a flat plate of aluminum and rivet like pin members made of aluminum material and for securing supporting the dial plate body to a time-keeping mechanism. The head portion of each pin member is formed so as to fit into a recess formed on the reverse surface of the body and being integrally fixed to the recess by means of ultrasonic wave welding. Also, a method of making the dial for the wrist watch is characterized in that when the head portion of the pin member is joined to the recess, a chip of the ultrasonic wave welding machine is pressure bonded to the head portion to provide the ultrasonic wave vibration so as to integrally join the head portion to the recess.

2 Claims, 13 Drawing Figures



PATENTED APR 16 1974

3,803,832

SHEET 1 OF 2

FIG - 1



FIG - 2



FIG - 3



FIG - 4



FIG - 5



FIG - 6



FIG - 7



PATENTED APR 16 1974

3,803,832

SHEET 2 OF 2

FIG - 8



FIG - 9



FIG - 10



FIG - 11



FIG - 12



FIG - 13



**DIAL FOR WRIST WATCH AND A METHOD OF  
MAKING THE SAME**

**SUMMARY OF INVENTION:**

The present invention relates to a dial structure for a wrist watch and to a method of making the same, and more particularly to a dial that is provided with a pin for securing the dial to a time-keeping mechanism and a method of joining the pin to the dial.

According to the broad concept of the present invention, the dial for the wrist watch comprises a dial body and a pin bonded to its reverse surface. The pin is inserted into a hole formed in the time-keeping mechanism and a set screw is urged against the pin in a right angle direction whereby the dial is fixed on the upper surface of the time-keeping mechanism.

The conventional dial is made of brass and a hollow pin is bonded by means of a soldering means. Thus the pin is soldered on the dial by soldering; for example, silver solder is sealed inside of the hollow pin and this pin is tack welded to the dial by spot welding. Thereafter the silver solder is melted by a burner or furnace, and the joint is formed by the application of the silver solder.

However, according to this welding method, there are disadvantages that not only involve the troublesome work of performing tack welding prior to the soldering, and also a substantial high degree technique is required. Further, there is considerable difficulty involved even if the pin is tack welded to the dial body nickel. The pin can easily be bent due to the high temperature heating action of the furnace or burner when the dial is fixed to the time-keeping mechanism, the bent pin obviously must be straightened. Further more, at the time of welding, the silver solder and flux flow as an integral body which leaves a convex mark on the periphery of the welded portion, and such a convex mark poses a problem when the dial is fixed to the time-keeping mechanism.

Also, the brass which is the material of the conventional dial has disadvantages such as it is more expensive than aluminum, its weight is heavier and also it has the difficulty of requiring forming work or surface treating and the like. Also, when the dial making involves electroplating with nickel, cyanide is used which is poisonous and which therefore is potentially harmful to the human body. Also, the residue therefrom may eventually flow to rivers which will become a public hazard.

On the other hand, heretofore, use of aluminum as the material in constructing the dial has been attempted. Even though the welding technique of aluminum is advanced, there is a distinct disadvantage that the strength of the dial is reduced during such process. The present status of the art is that efforts of making an aluminum dial of a high precision as a time-keeper part by a practical method has been unsuccessful. Additional disadvantages of this process are enumerated in the following; (1) when the pin is joined to the dial body by means of soldering, a convex mark is produced on the periphery of the welded portion as mentioned in the foregoing; (2) since the dial body is to be of a thin wall thickness and its volume is to be small, its structure and material necessarily become annealed by the heating action of soldering which results in a substantial remarkable loss of strength, and returning it to its original

strength is difficult; (3) although the foregoing disadvantage (2) can be eliminated if aluminum solder that melts at low temperature is used, in such a process alumite is formed and the aluminum solder and flux are not highly resistant to chemicals also erosion may occur and the joint portion of the pin tends to separate.

When aluminum is used as the material for the dial for the wrist watch, the foregoing disadvantages can be overcome. Further many advantages can be obtained with a dial made of aluminum as compared with the conventional dial made of brass. Some examples are (1) the dial can be made of a light weight; (2) the post or succeeding processing or treatment such as forming, surface coating and printing and the like can be easily performed; (3) desirable designs can be provided and (4) the dial can be constructed at low cost.

Under the circumstances as outlined above, the present inventor has confirmed, as a result of energetical studies, a method of making the dial for wrist watch method made of aluminum material which is free completely from the foregoing disadvantages.

The present invention is characterized in that the dial body is formed of aluminum material a recess is formed at a predetermined position on the body; a rivet like pin member is formed of aluminum or similar material; a head portion of the pin member fits into the recess; and the head portion and the recess are joined by the welding energy of an ultrasonic wave.

**BRIEF DESCRIPTION OF DRAWINGS:**

FIGS. 2 through 6 and FIGS. 8 through 12 show first and second embodiments, respectively, of the present invention;

FIG. 1 is a top plan view of the dial body;

FIG. 2 is a perspective view of the first embodiment of the pin;

FIG. 3 is an enlarged cross sectional view taken along line X — X of FIG. 1.

FIGS. 4 and 9 are cross sectional views of the dial and the pin before the pin is welded;

FIGS. 5 and 10 are cross sectional views of the condition where the pin is welded to the dial by the chip of the ultrasonic wave welding machine;

FIGS. 6 and 11 are bottom plan views, partially in section, of the dial body and the pin integrally welded together;

FIG. 7 is a cross sectional view showing one adverse example where the pin is welded to the dial body by the chip of the ultrasonic wave welding machine;

FIG. 8 is a perspective view of the second embodiment of the pin;

FIG. 12 is a cross sectional view of the chip used for welding the pin of the second embodiment to the dial plate; and

FIG. 13 is a cross sectional view of a structural arrangement wherein the dial is welded by the conventional method to the pin and the dial-pin unit is fixed to the time-keeping mechanism.

**PREFERRED EMBODIMENT OF THE INVENTION:**

Referring now to the accompanying drawings, two preferred embodiments of the invention will be described in detail with specific reference to FIGS. 2-6 and FIGS. 8-12, respectively. In FIG. 1, a circular flat dial plate 10 is provided with a circular center hole 11

and a rectangular aperture 12. As shown in FIG. 3 and FIG. 4, a circular recess 13 is formed in the vicinity of the periphery of the reverse surface of the dial body 10. The recess 13 is formed by measuring a predetermined position on the dial with the use of a jig for accurately positioning and by boring the recess with an endmill or dia. The pin 15 and the dial body 10 are secured to a time-keeping mechanism. The pin 15 is formed with a rivet like shape as shown in FIG. 2 is integrally provided with a head portion 14 of a flat circular shape, and is made of aluminum or similar material. The diameter of the head portion 14 is slightly smaller than the diameter of the recess 13, and also its wall thickness is equal to the depth of the recess 13 or is slightly shallower than the depth.

As shown in FIG. 5, in order to weld the pin 15 to the dial body 10, after fitting the head portion 14 to the recess 13, a hollow portion 16a of the chip 16 of the ultrasonic wave welding machine is inserted to operatively contact the pin 15. The tip portion of the chip 16 is operatively urged against the head portion 14, by the ultrasonic wave oscillation being applied thereto. When the oscillation is applied, the recess 13 and the head portion 14 are thereby welded integrally by the welding energy of the ultrasonic wave.

Since the pin 15 that is welded to the dial body 10 is employed for securing the dial to the time-keeping mechanism, it is required to have a high tensile strength and bending strength.

According to end results of an experiment conducted by the present inventor, a thickness of the head portion 14 was made 0.18 mm, its diameter was 0.9 mm, a diameter of the pin 15 was 0.65 mm, the pressure of the chip 16 for the head portion 14 was 5 kg, and its pressure contact time was 0.25 sec., the current of the ultrasonic wave welding machine was 2.5A, and the ultrasonic wave welding machine whose oscillating frequency was  $19.5 \pm KH_2$  was used; the pin 15 whose recess 13 was welded to the head portion 14 could withstand the tensile strength of 6 kg and also could withstand the bending strength (angle of 20°) of 15 times in the right and left directions or forward and backward directions, and such tensile strength and the bending strength having such values to substantially surpasses the tensile strength and bending strength ordinarily required for welding of the pin to the dial plate body.

In the present invention, the salient features are that, as mentioned in the foregoing, the recess 13 being provided in the dial plate body 10, the head portion 14 of the pin 15 being fitted and ultrasonically welded into the recess 13 whereby the joint surface of both elements can be made larger thus stronger. Also, with the foregoing arrangement, when the above-mentioned joining is made, there are advantages in that the erection of the pin 15 on the surface of the dial body 10 and the application of the pressure of the chip 16 to the pin 15 become extremely easy.

FIG. 6 illustrates the joining structure of 13 and the head portion 14. It can be recognized that a welded portion 17 is formed in ring shape and the reason for such form is that the tip portion of the chip 16 is formed in ring shape and thusly is made to correspond to the portion that is to be urged against. The pressure contacting portion produces a strong abrading action as compared with the other portion. In order to join not only the ring like welding portion 17 but also

the other portion, it may be considered that the pressure of the chip 16 against the head portion 14 can be made greater and its pressure contacting time can be prolonged. However the pressure and the pressure contacting time should not exceed certain maximum values. As shown in FIG. 7, there in such a situation, there is a possible adverse effect in that a bulged portion 18 can be formed on the periphery of the head portion 14. The bulged portion 18 becomes an obstacle in the case where the dial plate body 10 is fixed to the time-keeping mechanism. Also the convex mark whose shape can be similar to the head portion 14 is produced on the surface of the dial plate body 10, or the concave portion 13 is broken and the finish of the surface of the dial plate 10 becomes deteriorated.

As shown in FIG. 8, the pin 115 is provided with an enlarged diameter tapered neck portion 115a at the joint of the stem portion and the head portion 114. This enlarged neck portion does not become a problem when the dial body 110 is fixed to the time-keeping mechanism. The neck portion 115a plays a role of preventing the shearing off of the pin 115 from the stem portion of the pin 115 from the head portion 114 when the force of a fixed tensile and/or bending strength is applied to the pin 115. Namely, when the pin 115 is being welded to the dial body 10 the stem portion of the pin 115 may be sheared off from the head portion 114 when an excess tensile and/or the bending force is applied to the pin 115. However, with the pin 115 being an enlarged provided with neck portion 115a at its stem portion, there is a substantial increase in the tensile strength and bending strength as compared with the arrangement where the pin which is not provided the enlarged neck portion 115a.

Also, as shown in FIG. 9 and FIG. 10, the dial body 110 is provided with a different shaped surface in the recess, according to the second embodiment. A recess 113 is provided with a surface 113a whose center or medial section is elevated and is tapered from the medial section to the periphery of the recess. The projecting surface 113a produces abrading action that is necessary for its joining to the center surface of the head portion 114. Therefore when the required tensile and/or bending force is applied to the pin 115, it plays a role of preventing the shearing off of the head portion 114 from the concave portion 113. Namely, as described previously, the head portion 14 for the recess 13 may be sheared off from the recess 13 when an excess tensile and/or bending force is applied to the pin as the ring like portion 17 along is being integrally welded thereto. Where the recess 113 is provided with the surface 113a the necessary abrading action is produced on recess 113 and the center surface of the head portion 114 when the tip portion of the chip 116 is pressure contacted with the head portion 114. Therefore, as shown in FIG. 11, in addition to a welded portion 117, the welded portion 119 is formed on the center surface. As a result, the tensile and/or bending strength for the pin 115 becomes remarkably improved as compared with a recess that has not been provided with the projecting surface 113a.

In the present invention, the head portion 114 of the pin 115 being provided with an enlarged neck portion 115a can be welded to the recess 113. Also, the head portion of the pin 115 can be welded to the recess 113 that is provided with the surface 113a. Therefore, vari-

ous structural arrangements of the elements can be effected.

As shown in FIG. 10 and 12, the chip 116 has a structure which is substantially identical with that of the chip 16, with the exception that a tapered expanded portion 116b is provided at the tip of the hole whose shape is adapted to engage with the enlarged neck portion 115a.

In FIG. 13, the conventional dial 210 is provided with a pin 215. The pin 215 is made with a hollow shape, and inside thereof is sealed with silver solder 300. The pin 215 is welded to the dial 210 by means of the silver solder 300 the disadvantage of which has already been explained. The dial 210 having been mounted in contact with pin 215, as shown in FIG. 13, is then inserted in a time-keeping mechanism 301. A set screw 302 is pressure contacted with the pin 215 at right angles from the lateral direction whereby the pin is fixed to the time-keeping mechanism 301.

It is to be noted in the present invention that the dial bodies 10 and 110 may be made of an alloy whose principal component is aluminum which alloy can be welded by ultrasonic welding. Also instead of providing the tapered surface 113a on the recess 113, a portion whose shape is similar to the tapered surface 113a may be provided on the center surface of the head portion 114. Also, the present invention is not to be limited to the numerical values described in the foregoing description.

What is claimed is:

1. A dial structure for a wrist watch comprising in combination:

a dial body formed of a flat plate of aluminum and

having front and rear surfaces, said dial body having a plurality of circular recesses positioned on its rear surface adjacent the periphery thereof, each of said recesses having an inner surface continuously tapering from an elevated medial section to the periphery thereof; and

a plurality of circular rivet like pin members, each of said pin members formed of an aluminum material and having elongated stem and flat head portions, said stem portion integrally joined with said flat head portion and adapted to engage with a time keeping mechanism, said stem portion having an enlarged neck portion at the joint of said stem portion and said flat head portion, said enlarged tapered neck portion adapted to engage with an ultrasonic welding machine, said flat head portion of each of said pin members fixedly joining in a perpendicular manner with said elevated medial section of each of said inner surfaces of said recesses, respectively, of said dial body, said joint between said flat head portion and said elevated medial section adapted to be accomplished by the welding of said ultrasonic welding machine.

2. A dial structure for a wrist watch according to claim 5, wherein said enlarged neck portion tapers from a large cross sectional area at the joining peripheral line to a smaller cross sectional area a short distance from said joining peripheral line and said smaller cross sectional area at the connecting peripheral line between said neck portion and the body of said stem portion is substantially equal to the cross sectional area of the body of said stem portion.

\* \* \* \* \*